



US010124926B2

(12) **United States Patent**  
**Chung et al.**

(10) **Patent No.:** **US 10,124,926 B2**  
(b5) **Date of Patent:** **Nov. 13, 2018**

(54) **METHODS AND APPARATUS FOR  
MANUFACTURING FIBER-BASED,  
FOLDABLE PACKAGING ASSEMBLIES**

(71) Applicant: **Footprint International, LLC**,  
Scottsdale, AZ (US)

(72) Inventors: **Yoke Dou Chung**, Chandler, AZ (US);  
**Brandon Michael Moore**, Mesa, AZ  
(US); **Yiyun Zhang**, Gilbert, AZ (US)

(73) Assignee: **Footprint International, LLC**, Gilbert,  
AZ (US)

(\*) Notice: Subject to any disclaimer, the term of this  
patent is extended or adjusted under 35  
U.S.C. 154(b) by 112 days.

(21) Appl. No.: **15/221,174**

(22) Filed: **Jul. 27, 2016**

(65) **Prior Publication Data**

US 2018/0029766 A1 Feb. 1, 2018

(51) **Int. Cl.**

**B65D 5/50** (2006.01)  
**B65D 81/05** (2006.01)

(Continued)

(52) **U.S. Cl.**

CPC ..... **B65D 5/0069** (2013.01); **B65D 5/0005**  
(2013.01); **B65D 75/006** (2013.01); **B65D  
81/055** (2013.01); **B65D 81/057** (2013.01);  
**B65D 81/058** (2013.01); **B65D 2581/053**  
(2013.01); **B65D 2585/6837** (2013.01)

(58) **Field of Classification Search**

CPC ..... B65D 2581/058; B65D 2585/6837; B65D  
5/0005; B65D 5/5069; B65D 5/5071;  
B65D 81/05; B65D 81/053–81/058

See application file for complete search history.

(56)

**References Cited**

**U.S. PATENT DOCUMENTS**

3,081,018 A \* 3/1963 Hall ..... B65D 71/0096  
206/586

3,700,623 A 10/1972 Keim  
(Continued)

**FOREIGN PATENT DOCUMENTS**

EP 2492395 8/2012  
JP WO 2012117674 A1 \* 9/2012 ..... B65D 81/055

**OTHER PUBLICATIONS**

Stratasys's Molder Fiber products, information attached, also available at: <http://web.archive.org/web/20160709065240/www.stratasys.com/solutions/additive-manufacturing/tooling/molded-fiber/>.

(Continued)

*Primary Examiner* — Anthony Stashick

*Assistant Examiner* — Mollie Impink

(74) *Attorney, Agent, or Firm* — Jenning Strouss; Michael K. Kelly; Daniel R. Pote

(57)

**ABSTRACT**

Methods and systems for shipping original design manufacturer (ODM) boxes. The system includes: a plurality of corner sets, each comprising at least two fiber cushions; a plurality of end cap sets, each comprising two opposing corrugated sleeves; and a graphical guide comprising an end cap selector and a corner selector. The graphical guide is configured to allow a user to: compare an ODM box to the end cap selector to thereby select one of the plurality of end cap sets; and compare the ODM box to the corner selector to thereby select one of the plurality of end corner sets. Each sleeve comprises a plurality of height score lines, a plurality of width score lines, and a support feature to stabilize the sleeve during folding.

**9 Claims, 43 Drawing Sheets**



## (51) Int. Cl.

**B65D 5/355** (2006.01)  
**B65D 75/00** (2006.01)

(56)

## References Cited

## U.S. PATENT DOCUMENTS

|                   |         |               |                        |
|-------------------|---------|---------------|------------------------|
| 4,162,729 A *     | 7/1979  | Kaiser .....  | B65D 5/5028<br>206/453 |
| 5,169,497 A       | 12/1992 | Sarkar et al. |                        |
| 6,168,015 B1      | 1/2001  | Shimizu       |                        |
| 6,576,089 B1      | 6/2003  | Sato          |                        |
| 6,592,718 B1      | 7/2003  | Wong Shing    |                        |
| 2003/0038054 A1 * | 2/2003  | Hurley .....  | B65D 81/056<br>206/586 |
| 2009/0043051 A1   | 2/2009  | Gu            |                        |
| 2012/0248101 A1 * | 10/2012 | Tumber .....  | B65D 81/05<br>220/1.5  |
| 2015/0020987 A1   | 1/2015  | Sealey        |                        |

## OTHER PUBLICATIONS

- Keiding, Inc. Molded Fiber Packaging, information attached, also available at: <http://www.keiding.com/molded-fiber/manufacturing-process/>.
- Grenidea Technologies PTE Ltd., "Improved Molded Fiber Manufacturing", European Patent Publication No. EP 1492926 B1, published Apr. 11, 2007.
- AFP Packaging's Thermoformed Fiber Products, information attached, also available at: [http://afpackaging.com:80/thermoformed-fiber-molded-pulp](http://web.archive.org/web/20160715012547/http://afpackaging.com:80/thermoformed-fiber-molded-pulp).
- Mohamed Naceur Belgacem & Antonio Pizzi, "Lignocellulosic Fibers and Wood Handbook: Renewable Materials for Today's

Environment", 2016, John Wiley & Sons, Hoboken, New Jersey, Image attached, full book available at: <https://books.google.com/books?id=jTL8CwAAQBAJ&printsec=frontcover#v=onepage&q&f=false>.

Liisa Ohlsson & Robert Federer, "Efficient Use of Fluorescent Whitening Agents and Shading Colorants in the Production of White Paper and Board", 2002, Specialty Chemicals Inc, South Africa, Attached, also available at: [http://www.tappa.co.za/archive/APPW2002>Title/Efficient\\_use\\_of\\_fluorescent\\_w/efficient\\_use\\_of\\_fluorescent\\_w.html](http://www.tappa.co.za/archive/APPW2002>Title/Efficient_use_of_fluorescent_w/efficient_use_of_fluorescent_w.html).

The Cellucon Trust, "Cellulosic Pulps, Fibres and Materials", 2000, Woodhead Publishing Limited, Cambridge CB1 6AH, England, Image attached, full book also available at: <https://books.google.com/books?id=xO2iAgAAQBAJ&printsec=frontcover#v=onepage&q&f=false>.

Fobchem's Alkyl Ketene Dimer (AKD WAX) information attached, also available at: [http://web.archive.org/web/20151029042937/http://www.fobchem.com:80/html\\_products/Alkyl-Ketene-Dimer%EF%BC%88AKD-WAAX%EF%BC%89.html#.W2SnUtVKhEY](http://web.archive.org/web/20151029042937/http://www.fobchem.com:80/html_products/Alkyl-Ketene-Dimer%EF%BC%88AKD-WAAX%EF%BC%89.html#.W2SnUtVKhEY).

Shandong Tiancheng Chemical Co., Ltd.'s AKD WAX, information attached, also available at: <http://www.yztianchengchem.com/en/index.php?m=content&c=index&a=show&catid=38&id=124>.

Ashland Chemicals, information attached, also available at: <https://www.ashland.com/products>.

Unidyne TG-8111 or Unidyne TG-8731 available from Daikin or World of Chemicals, information attached, also available at: <https://www.worldofchemicals.com/chemicals/chemical-properties/unidyne-tg-8111.html>.

Hercobond 6950 information attached, also available at: <https://solenis.com/en/industries/tissue-towel/innovations/hercobond-dry-strength-additives>.

Hercobond 6950 information attached, also available at: [http://www.sfm.state.or.us/CR2K\\_SubDB/MSDS/HERCOBOND\\_6950.PDF](http://www.sfm.state.or.us/CR2K_SubDB/MSDS/HERCOBOND_6950.PDF).

\* cited by examiner





FIG. 2



FIG. 3

400



FIG. 4



FIG. 5A



FIG. 5B



FIG. 6A



FIG. 6B

**FIG. 6C**



FIG. 7



FIG. 8



FIG. 9



FIG. 10



FIG. 11A



FIG. 11B



FIG. 12



FIG. 13



FIG. 14



FIG. 15



FIG. 16



FIG. 17



FIG. 18





FIG. 20



FIG. 21



FIG. 22

**FIG. 23**



FIG. 24



FIG. 25



FIG. 26



FIG. 27



FIG. 28



FIG. 29



FIG. 30



FIG. 31



FIG. 32



FIG. 33



FIG. 34



FIG. 35



FIG. 36



FIG. 37



FIG. 38



FIG. 39



FIG. 40



FIG. 41



FIG. 42



FIG. 43



FIG. 44





FIG. 47





FIG. 48



FIG. 49



FIG. 50



FIG. 51



FIG. 52



**METHODS AND APPARATUS FOR  
MANUFACTURING FIBER-BASED,  
FOLDABLE PACKAGING ASSEMBLIES**

TECHNICAL FIELD

The present invention relates, generally, to ecologically sustainable methods and apparatus for manufacturing containers and packaging materials and, more particularly, to the use of novel slurries for use in vacuum forming molded fiber products to replace plastics.

BACKGROUND

Pollution caused by single use plastic containers and packaging materials is epidemic, scarring the global landscape and threatening the health of ecosystems and the various life forms that inhabit them. Trash comes into contact with waterways and oceans in the form of bits of Styrofoam and expanded polystyrene (EPS) packaging, to-go containers, bottles, thin film bags and photo-degraded plastic pellets.

As this ocean trash accumulates it forms massive patches of highly concentrated plastic islands located at each of our oceans' gyres. Sunlight and waves cause floating plastics to break into increasingly smaller particles, but they never completely disappear or biodegrade. A single plastic micro-bead can be one million times more toxic than the water around it. Plastic particles act as sponges for waterborne contaminants such as pesticides. Fish, turtles and even whales eat plastic objects, which can sicken or kill them. Smaller ocean animals ingest tiny plastic particles and pass them on to us when we eat seafood.

Sustainable solutions for reducing plastic pollution are gaining momentum. However, continuing adoption requires these solutions to not only be good for the environment, but also competitive with plastics from both a performance and a cost standpoint. The present invention involves replacing plastics with revolutionary technologies in molded fiber without compromising product performance, within a competitive cost structure.

By way of brief background, molded paper pulp (molded fiber) has been used since the 1930s to make containers, trays and other packages, but experienced a decline in the 1970s after the introduction of plastic foam packaging. Paper pulp can be produced from old newsprint, corrugated boxes and other plant fibers. Today, molded pulp packaging is widely used for electronics, household goods, automotive parts and medical products, and as an edge/corner protector or pallet tray for shipping electronic and other fragile components. Molds are made by machining a metal tool in the shape of a mirror image of the finished package. Holes are drilled through the tool and then a screen is attached to its surface. The vacuum is drawn through the holes while the screen prevents the pulp from clogging the holes.

The two most common types of molded pulp are classified as Type 1 and Type 2. Type 1 is commonly used for support packaging applications with  $\frac{3}{16}$  inch (4.7 mm) to  $\frac{1}{2}$  inch (12.7 mm) walls. Type 1 molded pulp manufacturing, also known as "dry" manufacturing, uses a fiber slurry made from ground newsprint, kraft paper or other fibers dissolved in water. A mold mounted on a platen is dipped or submerged in the slurry and a vacuum is applied to the generally convex backside. The vacuum pulls the slurry onto the mold to form the shape of the package. While still under the vacuum, the mold is removed from the slurry tank, allowing the water to drain from the pulp. Air is then blown through

the tool to eject the molded fiber piece. The part is typically deposited on a conveyor that moves through a drying oven.

Type 2 molded pulp manufacturing, also known as "wet" manufacturing, is typically used for packaging electronic equipment, cellular phones and household items with containers that have 0.02 inch (0.5 mm) to 0.06 inch (1.5 mm) walls. Type 2 molded pulp uses the same material and follows the same basic process as Type 1 manufacturing up to the point where the vacuum pulls the slurry onto the mold. After this step, a transfer mold mates with the fiber package on the side opposite of the original mold, moves the formed "wet part" to a hot press, and compresses and dries the fiber material to increase density and provide a smooth external surface finish. See, for example, <http://www.stratasys.com/solutions/additive-manufacturing/tooling/molded-fiber>; <http://www.keiding.com/molded-fiber/manufacturing-process/>; Grenidea Technologies PTE Ltd. European Patent Publication Number EP 1492926 B1 published Apr. 11, 2007 and entitled "Improved Molded Fiber Manufacturing"; and <http://afpackaging.com/thermoformed-fiber-molded-pulp/>. The entire contents of all of the foregoing are hereby incorporated by this reference.

Fiber-based packaging products are biodegradable, compostable and, unlike plastics, do not migrate into the ocean. However, presently known fiber technologies are not well suited for use with meat and poultry containers, prepared food, produce, microwavable food containers, and lids for beverage containers such as hot coffee.

Methods and apparatus are thus needed which overcome the limitations of the prior art.

Various features and characteristics will also become apparent from the subsequent detailed description and the appended claims, taken in conjunction with the accompanying drawings and this background section.

BRIEF SUMMARY

Various embodiments of the present invention relate to methods, chemical formulae, and apparatus for manufacturing vacuum molded, fiber-based packaging and container products including, *inter alia*: i) meat, produce, horticulture, and utility containers embodying novel geometric features which promote structural rigidity; ii) meat, produce, horticulture containers having embedded and/or topical moisture/vapor barriers; iii) vacuum tooling modified to re-direct spray nozzles to increase the size of vent holes in produce and horticulture containers; iv) microwavable/oven-heated containers embodying embedded and/or topical moisture, oil, and/or vapor barriers, and/or retention aids to improve chemical bonding; v) meat containers embodying a moisture/vapor barrier which preserves structural rigidity over an extended shelf life; vi) lids for hot beverage containers embodying a moisture/vapor barrier; vii) vacuum tooling modified to include a piston for ejecting beverage lids having a negative draft from the mold; and viii) a packaging kit for shipping flat screen televisions and other electronics.

It should be noted that the various inventions described herein, while illustrated in the context of conventional slurry-based vacuum form processes, are not so limited. Those skilled in the art will appreciate that the inventions described herein may contemplate any fiber-based manufacturing modality, including 3D printing techniques.

Various other embodiments, aspects, and features are described in greater detail below.

## BRIEF DESCRIPTION OF THE DRAWING FIGURES

Exemplary embodiments will hereinafter be described in conjunction with the appended drawing figures, wherein like numerals denote like elements, and:

FIG. 1 is a schematic block diagram of an exemplary vacuum forming process using a fiber-based slurry in accordance with various embodiments;

FIG. 2 is a schematic block diagram of an exemplary closed loop slurry system for controlling the chemical composition of the slurry in accordance with various embodiments;

FIG. 3 is a perspective view of an exemplary produce container depicting a rolled edge, overhanging skirt, and ribbed structural features for enhancing hoop strength in accordance with various embodiments;

FIG. 4 is an end view of the container shown in FIG. 3 in accordance with various embodiments;

FIG. 5A is a perspective view of an exemplary produce container including extended vent holes in accordance with various embodiments;

FIG. 5B is an end view of the container shown in FIG. 5A in accordance with various embodiments;

FIGS. 6A-6C are alternate embodiments of food containers illustrating various shelf and rib features in accordance with various embodiments;

FIG. 7 is a perspective view of an exemplary rinsing tool including spray nozzles configured to rinse pulp from vent hole inserts in accordance with various embodiments;

FIG. 8 is a close up view of the spray nozzles shown in FIG. 7 in accordance with various embodiments;

FIG. 9 is a perspective view of the excess fiber targeted for removal by the spray nozzles shown in FIGS. 7 and 8 in accordance with various embodiments;

FIG. 10 is a perspective view of an exemplary microwavable food container in accordance with various embodiments;

FIG. 11A is a perspective view of an exemplary meat container in accordance with various embodiments;

FIG. 11B is an end view of the microwavable food container shown in FIG. 11A in accordance with various embodiments;

FIG. 12 is an alternative embodiment of a shallow food tray illustrating a shelf having off-set ribs in accordance with various embodiments;

FIG. 13 is a perspective view of an exemplary lid for a liquid (e.g., soup or a beverage such as coffee or soda) container in accordance with various embodiments;

FIG. 14 is a top view of the lid shown in FIG. 13 in accordance with various embodiments;

FIG. 15 is a side elevation view of the lid shown in FIGS. 13 and 14 in accordance with various embodiments;

FIG. 16 is a perspective view of an exemplary mold for use in manufacturing the lid shown in FIGS. 13-15 in accordance with various embodiments;

FIG. 17 is a side elevation view of the mold of FIG. 16 shown in the retracted position in accordance with various embodiments;

FIG. 18 is a side elevation view of mold of FIG. 17 shown in the extended position in accordance with various embodiments;

FIG. 19 is a perspective view of utility (non-food) container in accordance with various embodiments;

FIG. 20 is a perspective view of a shipping kit for flat screen televisions and other electronics and fragile components in accordance with various embodiments;

FIGS. 21-35 are schematic perspective views of a telescopic packaging assembly for shipping big screen televisions in accordance with various embodiments; and

FIGS. 36-52 depict an alternative “end cap” technique for packaging ODM boxes in accordance with various embodiments.

## DETAILED DESCRIPTION OF PREFERRED EXEMPLARY EMBODIMENTS

The following detailed description of the invention is merely exemplary in nature and is not intended to limit the invention or the application and uses of the invention. Furthermore, there is no intention to be bound by any theory presented in the preceding background or the following detailed description.

Various embodiments of the present invention relate to fiber-based or pulp-base products for use both within and outside of the food and beverage industry. By way of non-limiting example, the present disclosure relates to particular chemical formulations of slurries adapted to address the unique challenges facing the food industry including oil barriers, moisture barriers, and water vapor barriers, and retention aids, the absence of which have heretofore prevented fiber-based products from displacing single use plastic containers and components in the food industry. The present disclosure further contemplates fiber-based containers having geometric and structural features for enhanced rigidity. Coupling these features with novel chemistries enables fiber-based products to replace their plastic counterparts in a wide variety of applications such as, for example: frozen, refrigerated, and non-refrigerated foods; medical, pharmaceutical, and biological applications; microwavable food containers; beverages; comestible and non-comestible liquids; substances which liberate water, oil, and/or water vapor during storage, shipment, and preparation (e.g., cooking); horticultural applications including consumable and landscaping/gardening plants, flowers, herbs, shrubs, and trees; chemical storage and dispensing apparatus (e.g., paint trays); produce (including human and animal foodstuffs such as fruits and vegetables); salads; prepared foods; packaging for meat, poultry, and fish; lids; cups; bottles; guides and separators for processing and displaying the foregoing; edge and corner pieces for packing, storing, and shipping electronics, mirrors, fine art, and other fragile components; buckets; tubes; industrial, automotive, marine, aerospace and military components such as gaskets, spacers, seals, cushions, and the like; and associated molds, wire mesh forms, recipes, processes, chemical formulae, tooling, slurry distribution, chemical monitoring, chemical infusion, and related systems, apparatus, methods, and techniques for manufacturing the foregoing components.

Referring now to FIG. 1, an exemplary vacuum forming system and process 100 using a fiber-based slurry includes a first stage 101 in which mold (not shown for clarity) in the form of a mirror image of the product to be manufactured is enveloped in a thin wire mesh form 102 to match the contour of the mold. A supply 104 of a fiber-based slurry 104 is input at a pressure (P1) 106 (typically ambient pressure). By maintaining a lower pressure (P2) 108 inside the mold, the slurry is drawn through the mesh form, trapping fiber particles in the shape of the mold, while evacuating excess slurry no for recirculation back into the system.

With continued reference to FIG. 1, a second stage 103 involves accumulating a fiber layer 130 around the wire mesh in the shape of the mold. When the layer 130 reaches a desired thickness, the mold enters a third stage 105 for

either wet or dry curing. In a wet curing process, the formed part is transferred to a heated hot press (not shown) and the layer 130 is compressed and dried to a desired thickness, thereby yielding a smooth external surface finish for the finished part. In a dry curing process, heated air is passed directly over the layer 130 to remove moisture therefrom, resulting in a more textured finish much like a conventional egg carton.

In accordance with various embodiments the vacuum mold process is operated as a closed loop system, in that the unused slurry is re-circulated back into the bath where the product is formed. As such, some of the chemical additives (discussed in more detail below) are absorbed into the individual fibers, and some of the additive remains in the water-based solution. During vacuum formation, only the fibers (which have absorbed some of the additives) are trapped into the form, while the remaining additives are re-circulated back in vacuum tank. Consequently, only the additives captured in the formed part must be replenished, as the remaining additives are re-circulated with the slurry in solution. As described below, the system maintains a steady state chemistry within the vacuum tank at predetermined volumetric ratios of the constituent components comprising the slurry.

Referring now to FIG. 2, is a closed loop slurry system 200 for controlling the chemical composition of the slurry. In the illustrated embodiment a tank 202 is filled with a fiber-based slurry 204 having a particular desired chemistry, whereupon a vacuum mold 206 is immersed into the slurry bath to form a molded part. After the molded part is formed to a desired thickness, the mold 206 is removed for subsequent processing 208 (e.g., forming, heating, drying, top coating, and the like).

In a typical wet press process, the Hot Press Temperature Range is around 150-250 degree C., with a Hot Press Pressure Range around 140-170 kg/cm<sup>2</sup>. The final product density should be around 0.5-1.5 g/cm<sup>3</sup>, and most likely around 0.9-1.1 g/cm<sup>3</sup>. Final product thickness is about 0.3-1.5 mm, and preferably about 0.5-0.8 mm.

With continued reference to FIG. 2, a fiber-based slurry comprising pulp and water is input into the tank 202 at a slurry input 210. In various embodiments, a grinder may be used to grind the pulp fiber to create additional bonding sites. One or more additional components or chemical additives may be supplied at respective inputs 212-214. The slurry may be re-circulated using a closed loop conduit 218, adding additional pulp and/or water as needed. To maintain a steady state balance of the desired chemical additives, a sampling module 216 is configured to measure or otherwise monitor the constituent components of the slurry, and dynamically or periodically adjust the respective additive levels by controlling respective inputs 212-214. Typically the slurry concentration is around 0.1-1%, most ideally around 0.3-0.4%. In one embodiment, the various chemical constituents are maintained at a predetermined desired percent by volume; alternatively, the chemistry may be maintained based on percent by weight or any other desired control modality.

The pulp fiber used in 202 can also be mechanically grinded to improve fiber-to-fiber bonding and improve bonding of chemicals to the fiber. In this way the slurry undergoes a refining process which changes the freeness, or drainage rate, of fiber materials. Refining physically modifies fibers to fibrillate and make them more flexible to achieve better bonding. Also, the refining process can increase tensile and burst strength of the final product. Freeness, in various embodiments, is related to the surface

conditions and swelling of the fibers. Freeness (csf) is suitably within the range of 200-700, and preferably about 220-250 for many of the processes and products described herein.

5 The chemical formulae (sometimes referred to herein as “chemistries”) and product configurations for various fiber-based packages and containers, as well as their methods for manufacture, will now be described in conjunction with FIGS. 3-19.

10

### Produce Containers

15 FIG. 3 is a perspective view of an exemplary produce container (e.g., mushroom till) 300 depicting a rolled edge 302, overhanging skirt 304, and various structural features including side ribs 306 and bottom ribs 308 for enhancing hoop strength. In this context, the term hoop strength refers to a measure of the applied lateral force along opposing vectors 310 versus the resulting deflection. Although the initial hoop strength of a container is primarily a function of 20 geometry, hoop strength tends to degrade as the container absorbs moisture liberated leached from its contents (e.g., mushrooms). The present inventor has determined that coupling various geometric features with slurry chemistries optimized for various applications can sustain hoop strength over extended shelf times. That is, by incorporating a moisture repellent barrier into the slurry (and/or applying a moisture repellent surface coating), the hoop strength may be maintained for a longer period of time even as the container contents bleed moisture.

25 FIG. 4 is an end view of a container 400 generally analogous to the container shown in FIG. 3, and illustrates a width dimension 402, a height dimension 404, and a skirt length 408 in the range of 0.1 to 5 millimeters, and preferably about 1.5 mm. In the illustrated embodiment, the skirt extends downwardly; alternatively, the skirt may extend at an oblique or obtuse angle relative to a vertical plane. Width and height dimensions 402, 404 may be any desired values, for example in the range of 20 to 400 mm, and preferably about 60 to 200 mm.

30 As briefly mentioned above, the various slurries used to vacuum mold containers according to the present invention comprises a fiber base mixture of pulp and water, with added chemical components to impart desired performance characteristics tuned to each particular product application. The 35 base fiber may include any one or combination of at least the following materials: softwood (SW), bagasse, bamboo, old corrugated containers (OCC), and newsprint (NP). Alternatively, the base fiber may be selected in accordance with the following resources, the entire contents of which are hereby incorporated by this reference: “Lignocellulosic Fibers and Wood Handbook: Renewable Materials for Today’s Environment,” edited by Mohamed Naceur Belgacem and Antonio Pizzi (Copyright 2016 by Scrivener Publishing, LLC) and available at <https://books.google.com/book?id=jTL8CwAAQBAJ&printsec=frontcover&v=onepage&g=false>; “Efficient use of Fluorescent Whiting Agents and Shading Colorants in the Production of White Paper and Board” by Liisa Ohlsson and Robert Federe, Published Oct. 8, 2002 in the African Pulp and Paper Week and available at [http://www.tappa.co.za/archive/APPW2002/Title/Efficient\\_use\\_of\\_fluorescent\\_w/efficient\\_use\\_of\\_fluorescent\\_w.html](http://www.tappa.co.za/archive/APPW2002/Title/Efficient_use_of_fluorescent_w/efficient_use_of_fluorescent_w.html); Cellulosic Pulps, Fibres and Materials: Cellucon '98 Proceedings, edited by J F Kennedy, G O Phillips, P A Williams, copyright 200 by Woodhead Publishing Ltd. and available at <https://books.google.com/books?id=xO2iAgAAQBAJ&printsec=frontcover&v=onepage&q=false>;

40 45 50 55 60 65

and U.S. Pat. No. 5,169,497 A entitled "Application of Enzymes and Flocculants for Enhancing the Freeness of Paper Making Pulp" issued Dec. 8, 1992.

For vacuum molded produce containers manufactured using either a wet or dry press, a fiber base of OCC and NP may be used, where the OCC component is between 50%-100%, and preferably about 70% OCC and 30% NP, with an added moisture/water repellent in the range of 1%-10% by weight, and preferably about 1.5%-4%, and most preferably about 4%. In a preferred embodiment, the moisture/water barrier may comprise alkylketene dimer (AKD) (for example, AKD 80) and/or long chain diketenes, available from FOBCHEM at [@.CozozvkrKUk](http://www.fobchem.com/html_products/Alkyl-Ketene-Dimer%EF%BC%88AKD-WAX%EF%BC%89.html); and Yanzhou Tiancheng Chemical Co., Ltd. at <http://www.yztianchengchem.com/en/index.php?m=content&c=index&a=show&catid=38&id=124&gclid=CPbn65aUg80CFRCOaQodoJUGRg>.

In order to yield specific colors for molded pulp products, cationic dye or fiber reactive dye may be added to the pulp. Fiber reactive dyes, such as Procion MX, bond with the fiber at a molecular level, becoming chemically part of the fabric. Also, adding salt, soda ash and/or increase pulp temperature will help the absorbed dye to be furtherly locked in the fabric to prevent color bleeding and enhance the color depth.

To enhance structural rigidity, a starch component may be added to the slurry, for example, liquid starches available commercially as Topcat® L98 cationic additive, Hercobond, and Topcat® L95 cationic additive (available from Penford Products Co. of Cedar Rapids, Iowa). Alternatively, the liquid starch can also be combined with low charge liquid cationic starches such as those available as Penbond® cationic additive and PAF 9137 BR cationic additive (also available from Penford Products Co., Cedar Rapids, Iowa).

For dry press processes, Topcat L95 may be added as a percent by weight in the range of 0.5%-10%, and preferably about 1%-7%, and particularly for products which need maintain strength in a high moisture environment most preferably about 6.5%; otherwise, most preferably about 1.5-2.0%. For wet press processes, dry strength additives such as Topcat L95 or Hercobond which are made from modified polyamines that form both hydrogen and ionic bonds with fibers and fines. Those additives may be added as a percent by weight in the range of 0.5%-10%, and preferably about 1%-6%, and most preferably about 3.5%. In addition, wet processes may benefit from the addition of wet strength additives, for example solutions formulated with polyamide-epichlorohydrin (PAE) resin such as Kymene 577 or similar component available from Ashland Specialty Chemical Products at <http://www.ashland.com/products>. In a preferred embodiment, Kymene 577 may be added in a percent by volume range of 0.5%-10%, and preferably about 1%-4%, and most preferably about 2%. Kymene 577 is of the class of polycationic materials containing an average of two or more amino and/or quaternary ammonium salt groups per molecule. Such amino groups tend to protonate in acidic solutions to produce cationic species. Other examples of polycationic materials include polymers derived from the modification with epichlorohydrin of amino containing polyamides such as those prepared from the condensation adipic acid and dimethylene triamine, available commercially as Hercosett 57 from Hercules and Catalyst 3774 from Ciba-Geigy.

In some packaging applications it is desired to allow air to flow through the container, for example, to facilitate ripening or avoid spoliation of the contents (e.g. tomatoes). However, conventional vacuum tooling typically rinses

excess fiber from the mold using a downwardly directed water spray, thereby limiting the size of the resulting vent holes in the finished produce. The present inventor has determined that re-directing the spray facilitates greater fiber removal during the rinse cycle, producing a larger vent hole in the finished product for a given mold configuration.

More particularly, FIG. 5A is a perspective view of an exemplary produce container 500 including extended relief holes 502. FIG. 5B is an end view of a container 504 illustrating extended vent holes 506. In this context, the term "extended vent holes" refers to holes made using the modified tooling shown in FIGS. 9-7, discussed below.

Referring now to FIGS. 6A-6C, various combinations of geometric features may be employed to enhance the structural rigidity/integrity of food containers. By way of non-limiting example, one or more horizontally extending shelves 602, 604 may be disposed between an upper region and a lower region of a side wall. For side walls containing a single shelf, the shelf may be disposed in the range of 30%-50% of the wall height from the top of the tray, and preferably about 35%. The shelf may be created by indenting the side panel and/or varying the draft angle. For example, in the embodiment shown in FIG. 6C, a lower region 606 exhibits a draft angle in the range of about 4-6° (and preferably about 5°), while an upper region 608 exhibits a draft angle in the range of about 6-8° (and preferably about 7°).

With continued reference to FIGS. 6A-6C, various rib configurations 610 may be disposed along the bottom and up the side panels of food containers. Ribs may be configured to terminate at a shelf, above the shelf (e.g., in the upper region of a side wall, for example 25% of the distance down from the top edge), below the shelf (e.g., in the lower region of a side wall, for example 25% of the distance down from the shelf), or at the top edge of the side wall. As shown in FIG. 6C, ribs 612 may extend from the bottom of the container upwardly and terminate at the shelf, whereupon subsequent ribs 614 may be offset from the ribs 612 and extend upwardly from the shelf. The ribs may terminate in a rounded, squared, or other desired geometrical shape or configuration.

#### Vent Hole Tooling

FIG. 7 is a directional water impingement cleaning system 700 including a plurality of re-directed spray nozzles 704 configured to rinse excess pulp from vent hole inserts 706. More particularly, a mold (not shown) is covered by a wire mesh 708, the mold including the inserts which correspond to vent holes in the finished product. A supply conduit 702 distributes rinse water to a manifold 711 which includes a plurality of spray nozzles, each configured to direct rinse water to remove excess fiber proximate the inserts.

With momentary reference to FIG. 8, a close up view 800 of a section of a manifold 811 depicts a spray nozzle 802 configured to direct rinse water proximate a corresponding insert 706. In this way, a greater extent of the residual fibers surrounding the inserts is removed, resulting in extended vent holes in the finished produce vis-à-vis presently known systems which simply rinse the mold with water sprayed from above. Importantly, the extended vent holes may be realized without having to adjust the underlying mold or inserts.

As seen in FIG. 9, the excess fiber 900 targeted for removal by the improved spray nozzles of the present invention provides extended vent holes using existing molds and presently known inserts.

## Microwavable Containers

Building on knowledge obtained from the development of the aforementioned produce containers, the present inventor has determined that molded fiber containers can be rendered suitable as single use food containers suitable for use in microwave, convection, and conventional ovens by optimizing the slurry chemistry. In particular, the slurry chemistry should advantageously accommodate one or more of the following three performance metrics: i) moisture barrier; ii) oil barrier; and iii) water vapor (condensation) barrier to avoid condensate due to placing the hot container on a surface having a lower temperature than the container. In this context, the extent to which water vapor permeates the container is related to the porosity of the container, which the present invention seeks to reduce. That is, even if the container is effectively impermeable to oil and water, it may nonetheless compromise the user experience if water vapor permeates the container, particularly if the water vapor condenses on a cold surface, leaving behind a moisture ring. The present inventor has further determined that the condensate problem is uniquely pronounced in fiber-based applications because water vapor typically does not permeate a plastic barrier.

Accordingly, for microwavable containers the present invention contemplates a fiber or pulp-based slurry including a water barrier, oil barrier, and water vapor barrier, and an optional retention aid. In an embodiment, a fiber base of softwood (SW)/bagasse at a ratio in the range of about 10%-90%, and preferably about 7:3 may be used. As a moisture barrier, AKD may be used in the range of about 0.5%-10%, and preferably about 1.5%-4%, and most preferably about 3.5%. As an oil barrier, the grease and oil repellent additives are usually water based emulsions of fluorine containing compositions of fluorocarbon resin or other fluorine-containing polymers such as UNIDYNE TG 8111 or UNIDYNE TG-8731 available from Daikin or World of Chemicals at <http://www.worldofchemicals.com/chemicals/chemical-properties/unidyne-tg-8111.html>. The oil barrier component of the slurry (or topical coat) may comprise, as a percentage by weight, in the range of 0.5%-10%, and preferably about 1%-4%, and most preferably about 2.5%. As a retention aid, an organic compound such as Nalco 7527 available from the Nalco Company of Naperville, Ill. May be employed in the range of 0.1%-1% by volume, and preferably about 0.3%. Finally, to strengthen the finished product, a dry strength additive such as an inorganic salt (e.g., Hercobond 6950 available at <http://solenis.com/en/industries/tissue-towel/innovations/hercobond-dry-strength-additives/>; see also [http://www.sfm.state.or.us/CR2K\\_SubDB/MSDS/HERCOBOND\\_6950.PDF](http://www.sfm.state.or.us/CR2K_SubDB/MSDS/HERCOBOND_6950.PDF)) may be employed in the range of 0.5%-10% by weight, and preferably about 1.5%-5%, and most preferably about 4%.

Referring now to FIG. 10, an exemplary microwavable food container 1000 depicts two compartments; alternatively, the container may comprise any desired shape (e.g., a round bowl, elliptical, rectangular, or the like). As stated above, the various water, oil, and vapor barrier additives may be mixed into the slurry, applied topically as a spray or coating, or both.

## Meat Containers

Presently known meat trays, such as those used for the display of poultry, beef, pork, and seafood in grocery stores, are typically made of plastic based materials such as poly-

styrene and Styrofoam, primarily because of their superior moisture barrier properties. The present inventor has determined that variations of the foregoing chemistries used for microwavable containers may be adapted for use in meat trays, particularly with respect to the moisture barrier (oil and porosity barriers are typically not as important in a meat tray as they are in a microwave container).

Accordingly, for meat containers the present invention contemplates a fiber or pulp-based slurry including a water barrier and an optional oil barrier. In an embodiment, a fiber base of softwood (SW)/bagasse and/or bamboo/bagasse at a ratio in the range of about 10%-90%, and preferably about 7:3 may be used. As a moisture/water barrier, AKD may be used in the range of about 0.5%-10%, and preferably about 1%-4%, and most preferably about 4%. As an oil barrier, a water based emulsion may be employed such as UNIDYNE TG 8111 or UNIDYNE TG-8731. The oil barrier component of the slurry (or topical coat) may comprise, as a percentage by weight, in the range of 0.5%-10%, and preferably about 1%-4%, and most preferably about 1.5%. Finally, to strengthen the finished product, a dry strength additive such as Hercobond 6950 may be employed in the range of 0.5%-10% by weight, and preferably about 1.5%-4%, and most preferably about 4%.

As discussed above in connection with the produce containers, the slurry chemistry may be combined with structural features to provide prolonged rigidity over time by preventing moisture/water from penetrating into the tray.

FIG. 11A is a perspective view of an exemplary meat container 1100, and FIG. 11B is an end view of the meat container shown in FIG. 11A including sidewall ribs 1102 and bottom ribs 1104.

FIG. 12 is a perspective view of an exemplary shallow meat container 1200 including a rib 1202 extending along the bottom and upwardly along the side wall, terminating at a shelf 1204. A second rib 1206, offset from the first rib 1202, extends upwardly from the shelf.

## Beverage Lids

Although fiber and pulp based paper cups are widely known, the beverage industry still needs a sustainable fiber-based lid solution. A significant impediment to the widespread adoption of fiber-based lids surrounds the ability to incorporate a zero or negative draft into the lid, in a manner which allows it to be conveniently removed from the mold. In addition, the fiber-based chemistry must be adapted to provide an adequate moisture/water barrier so that the rigidity of the lid is not compromised in the presence of liquid. The methods, chemical formulae, and tooling contemplated by the present invention addresses both of these issues in a manner heretofore not addressed by the prior art.

In particular, the chemistry for lids is similar to meat trays and microwave bowls discussed above. Specifically, for beverage container lids the present invention contemplates a fiber or pulp-based slurry including a water/moisture barrier and an optional retention aid. In an embodiment, a fiber base of softwood (SW)/bagasse and/or bamboo/bagasse at a ratio in the range of about 10%-90%, and preferably about 7:3 may be used. As a moisture/water barrier, AKD may be used in the range of about 0.5%-10%, and preferably about 1%-4%, and most preferably about 4%. Rigidity may be enhanced by Hercobond 6950 in the range of 0.5%-10% by weight, and preferably about 1%-4%, and most preferably about 2%. Kymene may also be added in the range of 0.5%-10%, and preferably about 1%-4%, and most preferably about 3%.

## 11

Referring now to FIG. 13, an exemplary lid 1300 includes an inclined platform 1302 surrounded by a retaining wall 1303 designed to urge liquid which leaves the inside of the container toward a sip hole 1304. A small venting aperture 1310 may be disposed on the platform 1302. A crown 1306 defines a volumetric space between the top of the cup (not shown) and the platform 1302, and a lock ring 1308 is configured to securely snap around the top of the cup. FIG. 14 is a top view of the lid shown in FIG. 13, including a platform 1402 venting aperture 1410, and sip hole 1404 for comparison.

FIG. 15 is a side elevation view of a lid 1500, highlighting a negative draft 1522 associated with the lock ring. Conventional wisdom suggests that vacuum molded products may not embody zero or negative draft features, because conventional vacuum mold tooling does not allow the finished part to be removed from the tool, in as much as the negative draft feature would “lock” the part to the tool in much the same way as the finished part “locks” itself to its mating component (here, the beverage cup). To overcome this limitation, the present invention contemplates a vacuum mold tool which removes the lid from the mold, notwithstanding the presence of the zero or negative draft locking feature, as described in greater detail below in conjunction with FIGS. 13-18.

## Lid Tooling

A tool for making a fiber-based lid having a zero or negative draft comprises a retractable piston having a shape which generally to a mirror image of the lid, and which is configured to extend to unlock the finished lid from that part of the mold which the lid locks to.

Referring now to FIG. 16, is a perspective view of an exemplary mold assembly for use in manufacturing the lid shown in FIGS. 13-15 in accordance with various embodiments. More particularly, a mold assembly 1600 includes a mold block 1620 supporting a lock ring mold portion 1608 (corresponding to the lock ring 1308 of FIG. 13), a retractable piston assembly comprising a crown portion 1630 having an inclined platform 1602 (corresponding to the inclined platform 1302 of FIG. 13), and a shaft portion 1640. In operation, a wire mesh (not shown) surrounds the piston assembly 1630 and lock ring portion 1608, and slurry is vacuum drawn through a series of holes 1650 to accumulate fiber around the wire mesh in the shape of the lid. In so doing, the lock ring 1308 of the lid locks around the lock ring mold portion 1608.

FIG. 17 is a side elevation view of the mold of FIG. 16 shown in the retracted position. In particular, the crown portion 1706 of the piston is adjacent the lock ring portion 1708 of the mold block 1720 when the piston is in the retracted position shown in FIG. 17. When the lid is formed around the wire mesh surrounding the mold form, the negative draft portion 1522 of the lid (see FIG. 15) locks around the corresponding negative draft portion 1722 of the lock ring portion 1708 of the mold. In order to remove the finished part from the mold, the piston is extended upwardly, forcing the lock ring of the lid to momentarily expand and unlock from the mold.

FIG. 18 shows the piston in the extended position. In particular, the shaft 1840 forces the crown portion 1830 away from the lock ring portion 1808, unlocking the lid from the negative draft feature 1822 of the mold. In an embodi-

## 12

ment, the piston is extended pneumatically, and allowed to retract by its own weight once the high pressure air is released.

## 5 Utility and Shipping Containers

FIG. 19 is a perspective view of utility (non-food) container 1900 including sidewall ribs 1902 and a perimeter lip 1904 in accordance with various embodiments. Depending on the nature of the contained material, any one or combination of the aforementioned chemistries may be used in the construction of the container. For example, if the contained liquid includes a water component, a suitable moisture/water barrier may be employed; if the contained material includes an oil component, a suitable oil barrier may be employed, and so on.

FIG. 20 is a perspective view of a shipping kit for flat screen televisions, computers, and other electronics and fragile components in accordance with various embodiments. By way of contrast, presently known shipping containers and protective packaging employ air bags, foam blocks, or foam filled bags. The present invention contemplates a bio-friendly, sustainable solution for shipping electronics in the form of a kit which may be used to send a flat screen TV returned by a consumer to a refurbishing center. In the illustrated embodiment, the kit includes: i) a top cover 2002 ii) a screen protector 2004; iii) four corrugated pulp corner pieces 2006 fitted over the corners of a flat screen TV 2008; iv) a bottom tray 2010; and v) one or more pallet straps 2012 for tying the finished assembly together.

FIGS. 21-35 illustrate methods and packing components for telescopically enclosing a large screen television, monitor, or other delicate (e.g., electronic, artistic, glass) equipment between left and right corrugated packing components. In various embodiments, the left and right packing components are telescopically aligned to accommodate shipped goods (e.g., TVs) having various lengths using a single, adjustable packaging assembly. Multiple score lines are placed near the top of each of the left and right corrugated components to accommodate different heights of TVs. The combination of the scored height adjustment and telescoping left and right packing components allows for a few packaging assemblies to accommodate a large number of different TV sizes.

Referring now to FIG. 21, a front view of a packaged assembly 2100 depicts a left telescopic end piece 2102 and a right telescopic end piece 2104. FIG. 22 shows the back side of the same assembly, with the left and right end pieces separated. FIG. 23 shows a subassembly 2300 including a TV 2301, a top cushion 2304, a bottom cushion 2306, and respective corner cushions 2302. The various cushion components may be vacuum formed from pulp according to the various embodiments described above. The manner in which the foregoing components may be manipulated into a packaged assembly will now be described in conjunction with FIGS. 24-35.

FIG. 24 shows an exemplary left end piece 2400 in the planar condition, prior to being folded into a sleeve. For reference, a bottom panel 2402 and an end panel 2404 are labeled in the figure. FIG. 25 shows a panel 2502 folded along an arrow 2504, and a panel 2506 folded along an arrow 2508. In FIG. 26, a panel 2602 is folded along an arrow 2604, and a panel 2608 folded along an arrow 2610. An interlocking section is suitably pushed through a corresponding hole, shown in window 2606, for added stability.

FIG. 27 illustrates a panel 2702 folded along an arrow 2704, whereupon the end piece is turned upside down and the bottom taped 2710. The foregoing process is repeated for the right end piece.

FIG. 28 is an exploded view of a package assembly 2800 including a flat screen 2801, a left end piece 2802, a right end piece 2804, a top cushion 2806, a bottom cushion 2808, and respective corner cushions 2810. In the illustrated embodiment, the flat screen and surrounding components are suitably inserted into the telescopically aligned end pieces such that the back side 2813 of the flat screen is exposed to an open back 2811 defined between the left and right end pieces. The manner in which the foregoing components are assembled into a final configuration for shipping will now be described in conjunction with FIGS. 29-35.

FIG. 29 illustrates an exemplary corner cushion 2900 including a concave part 2902 for receiving a corner of the flat screen, and a support part 2904 separated by a fold line 2906. The support part 2904 may be manually folded along the arrow 2908 into the folded position 2910. FIG. 30 shows the left and right sleeves 3002, 3004 being telescopically adjusted along the arrow 3001 to accommodate the length of the TV being packaged. FIG. 30 further depicts the two bottom folded corner pieces 2910 and bottom cushion 2808 being inserted into the aligned sleeves, as indicated by the arrows 3003.

FIG. 31 shows the TV being inserted into the assembled sleeves, followed by a final adjustment of the sleeves along arrow 3102 to ensure a snug fit, followed by the packing of the top corner cushions 2910 and top cushion 2806.

FIG. 32 shows respective end flaps 3202 being folded inward along arrows 3203. FIG. 32 shows top flaps 3302 being folded down along arrows 3303, and top flaps 3304 being folded down along arrows 3305. FIG. 34 shows the folded flaps being taped in place at positions 3402. FIG. 35 shows the packaged assembly being wrapped in stretch wrap 3502.

The present application also provides an environmentally responsible, sustainable solution for packaging flat screen televisions, monitors, and other delicate (e.g., electronic, artistic, glass) equipment already packed in its own box. This solution uses corrugated and fiber materials and, thus, avoids the use of non-renewable, single use plastics. In contrast to the telescopic configuration described above, the ensuing "end cap" solution provides a system for packaging rectangular boxes of virtually any size, using three different end cap sizes to accommodate different TV box heights, in combination with four different fiber corner cushions, using a sizing system which includes score lines on the end caps.

In an embodiment, each end cap comprises a rectangular corrugated component having two pulp cushions, and score lines for adjusting the height of the finished end cap. The end caps are placed on either end of the original design manufacturer (ODM) box. A corrugated screen protector assembly including fiber "feet" is placed over the top middle of the box to protect the underlying screen from breakage during shipment. The ODM box, along with the end caps, screen protector, and corner cushions, is then assembled and surrounded with stretch wrap or palette straps to hold the entire pack together.

Various methods and materials for packaging TVs using this end cap solution will now be described in conjunction with FIGS. 36-51.

FIG. 36 is an exploded view of an exemplary end cap solution including an ODM box 3601 with a TV inside, respective end caps 3602 and corner cushions 3604, and a corrugate screen protector assembly 3606 having one or

more molded fiber feet arrays 3610 disposed on an inside (screen facing) surface 3608 of the screen protector assembly.

FIG. 37 is a matrix guide mapping a plurality (e.g., four) of fiber cushion 3702 sizes to a plurality (e.g., three) of end cap 3704 sizes to yield a plurality of assembly configuration combinations 3706 (e.g., twelve).

FIG. 38 is a graphical guide 3800 for assisting shipping personnel in selecting the appropriate end caps and fiber corners for a given ODM box size according to the invention. In the illustrated embodiment the guide 3800 includes an end cap selector 3802 and a corner selector 3804.

FIG. 39 shows an ODM box 3901 being compared to the end cap selection guide 3802. In particular, the end cap selector includes a first zone 3902 corresponding to an end cap A, a second zone 3904 corresponding to an end cap B, and a third zone 3906 corresponding to an end cap C. by lining up the ODM box with the end cap guide, the user can visually determine whether an A, B, or C end cap should be selected.

FIG. 40 shows the ODM box being compared to the fiber corner guard selector 3804. Specifically, by lining up a right edge 4002 of the box with a guide line 4004 on the selector chart, the width 4006 of the box determines which one of a plurality of corner guard sizes should be selected for the particular box under inspection. Having selected the optimum end caps and the optimum corner guards, the manner in which they are assembled around the ODM box will now be described in conjunction with FIGS. 41-51.

FIG. 41 shows a planar corrugate 4100 prior to being folded into an end cap. The corrugate 4100 includes a plurality of height score lines 4110, width score lines 4112, and a support feature 4102 having one or more tabs 4104, 4106, described in greater detail below.

FIG. 42 illustrates how the support tabs facilitate taping the end cap flaps. In particular, the thickness of a corner cushion may be defined by dimension 4201. For a thinner cushion, the end cap may be folded along an inner score line 4204; for a thicker cushion, the end cap may be folded along an outer score line 4202. When using the outer score line, the side flap rests on an edge 4205 (with the tab 4206 bent at a 90° angle, as shown) during taping. However, when using the inner score line, the side flap does not rest on edge 4205, and thus may be unstable during the critical taping operation. Accordingly, when using the inner score line 4204, the tab 4206 is not bent, to thereby provide a stable support for the side flap during taping. Those skilled in the art will appreciate that and number of score lines and associated stepped tabs may be employed to provide stability when taping for any one of a plurality of corner guard thicknesses (and corresponding score lines).

Using the aforementioned support tabs, the bottom flaps may be taped together as shown in FIGS. 43 and 44. As shown in FIG. 45, a corner guard 4501 may then be placed in the bottom area of each end cap 4502.

FIG. 46 shows the ODM box 4601 being inserted into the respective end caps with the bottom corner guards (not shown) installed. FIGS. 47 and 48 illustrate the installation of the top corner guards. Note the plurality of height adjustment score lines 4802 on the top flaps of the end caps. FIG. 49 shows the end flaps being securely folded along the appropriate score lines over the corner guards.

FIG. 50 illustrates respective end caps 5002 secured to the ODM box 5001, whereupon a screen protector 5004 (having molded fiber feet, not shown) is installed over the box by folding the screen protector along appropriate score lines

## 15

**5003.** The final assembly may then be securely wrapped in stretch paper **5102** (FIG. **51**) or, alternatively, secured with pallet straps **5202** (FIG. **52**).

While the present invention has been described in the context of the foregoing embodiments, it will be appreciated that the invention is not so limited. For example, the various geometric features and chemistries may be adjusted to accommodate additional applications based on the teachings of the present invention.

A method is thus provided for manufacturing a produce container. The method includes: forming a wire mesh over a mold comprising a mirror image of the produce container; immersing the wire mesh in a fiber-based slurry bath; drawing a vacuum across the wire mesh to cause fiber particles to accumulate at the wire mesh surface; and removing the wire mesh from the slurry bath; wherein the slurry comprises a moisture/water barrier component in the range of 1.5%-4% by weight.

In an embodiment the slurry comprises a moisture barrier component in the range of about 4%.

In an embodiment the moisture barrier component comprises alkyltene dimer (AKD).

In an embodiment the moisture barrier component comprises alkyltene dimer (AKD) 80.

In an embodiment the slurry comprises a fiber base of OCC/NP at a ratio in the range of 0.5/9.5.

In an embodiment the slurry further comprises a starch component in the range of 1%-7% by weight.

In an embodiment the starch component comprises a cationic liquid starch.

In an embodiment the slurry further comprises a wet strength component such as Kymene (e.g., Kymene 577) in the range of 1%-4% by weight.

In an embodiment the mold comprises a rolled edge including a vertically descending skirt.

In an embodiment the moisture/water barrier comprises AKD in the range of about 4%; the slurry comprises a cationic liquid starch component in the range of 1%-7%; and the mold comprises a rolled edge including a vertically descending skirt, at least one bottom rib, and at least one sidewall rib.

A produce container manufactured according to the foregoing methods is also provided.

In a vacuum mold assembly of the type including a wire mesh surrounding a mold form having a substantially vertical insert configured to provide a vent hole in a finished container, a directional rinse assembly is provided. The directional rinse assembly includes: a water supply conduit; a manifold connected to the water supply conduit; and a spray nozzle connected to the manifold and configured to direct a spray of water at the insert along a vector having a horizontal component.

In an embodiment the mold includes a plurality of substantially vertical inserts, and the directional rinse assembly further includes a plurality of spray nozzles, each configured to direct a spray of water at respective inserts along respective vectors each having a horizontal component.

A method is also provided for manufacturing a zero or nearly zero porosity food container. This method includes a wet press procedure as the first step, followed by an extra surface coating procedure for applying a thin layer of water based long chain fluorine-containing polymers such as Daikin S 2066, in the range of about 0.5%-6% by weight, and preferably about 1%-5%, and most preferably about 4%.

A method is also provided for manufacturing a micro-wavable and/or oven worthy food container. The method includes: forming a wire mesh over a mold comprising a

## 16

mirror image of the microwavable food container; immersing the wire mesh in a fiber-based slurry bath; drawing a vacuum across the wire mesh to cause fiber particles to accumulate at the wire mesh surface; and removing the wire mesh from the slurry bath; wherein the slurry comprises a moisture barrier component in the range of 0.5%-10% by weight, an oil barrier in the range of 0.5%-10% by weight, and a retention aid in the range of 0.05%-5% by weight.

In an embodiment the moisture/water barrier component is in the range of about 1.5%-4%, the oil barrier is in the range of about 1%-4%, and the retention aid is in the range of about 0.1%-0.5%.

In an embodiment the moisture barrier component comprises alkyltene dimer (AKD).

In an embodiment the moisture barrier component comprises alkyltene dimer (AKD) 79.

In an embodiment the slurry comprises a fiber base of SW/bagasse at a ratio in the range of 0.5/9.5.

In an embodiment the slurry further comprises a rigidity component in the range of 1%-5% by weight.

In an embodiment the rigidity component comprises a dry inorganic salt.

In an embodiment the oil barrier comprises a water based emulsion.

In an embodiment the oil barrier comprises TG 8111.

In an embodiment the retention aid comprises an organic compound.

In an embodiment the retention aid comprises Nalco 7527.

In an embodiment the moisture/water barrier comprises AKD in the range of about 4%; the slurry comprises bagasse and a dry inorganic salt; the oil barrier comprises a water based emulsion; and the vapor barrier comprises an organic compound.

A microwavable container manufactured according to the foregoing methods is also provided.

A method of manufacturing a meat tray is provided, the method including: forming a wire mesh over a mold comprising a mirror image of the meat tray; immersing the wire mesh in a fiber-based slurry bath; drawing a vacuum across the wire mesh to cause fiber particles to accumulate at the wire mesh surface; and removing the wire mesh from the slurry bath; wherein the slurry comprises a moisture/water barrier component in the range of 0.5%-10% by weight and an oil barrier in the range of 0.5%-10% by weight.

In an embodiment the moisture/water barrier component is in the range of about 1%-4% and the oil barrier is in the range of about 1%-4%.

In an embodiment the moisture barrier component comprises alkyltene dimer (AKD).

In an embodiment the moisture barrier component comprises alkyltene dimer (AKD) 79.

In an embodiment the slurry comprises a fiber base of SW/bagasse at a ratio in the range of 1/9.

In an embodiment the slurry includes a rigidity component in the range of 1.5%-4% by weight.

In an embodiment the rigidity component comprises a dry inorganic salt.

In an embodiment the oil barrier comprises a water based emulsion.

In an embodiment the oil barrier comprises TG 8111 in the range of about 1.5% by weight.

In an embodiment the moisture/water barrier comprises AKD in the range of about 4%; the slurry comprises bagasse and a dry inorganic salt; and the oil barrier comprises a water based emulsion.

## 17

A meat tray manufactured according to the foregoing methods is also provided.

In an embodiment the meat tray includes at least one sidewall rib and at least one bottom rib.

A method of manufacturing a lid for a beverage container is also provided. The method includes: forming a wire mesh over a mold comprising a mirror image of the lid; immersing the wire mesh in a fiber-based slurry bath; drawing a vacuum across the wire mesh to cause fiber particles to accumulate at the wire mesh surface; and removing the wire mesh from the slurry bath; wherein the slurry comprises a moisture/water barrier component in the range of 0.5%-10% by weight, a rigidity component in the range of 1%-4% by weight, and a polycationic component in the range of about 1%-4%.

In an embodiment the moisture/water barrier component is in the range of about 1%-4% and the oil barrier is in the range of about 1%-4%.

In an embodiment the moisture barrier component comprises alkyltene dimer (AKD).

In an embodiment the moisture barrier component comprises alkyltene dimer (AKD) 80.

In an embodiment the slurry comprises a fiber base of SW/bagasse at a ratio in the range of 1/9.

In an embodiment the slurry further comprises a rigidity component in the range of 1%-4% by weight.

In an embodiment the rigidity component comprises a dry inorganic salt.

In an embodiment the moisture/water barrier comprises AKD in the range of about 4%; the slurry comprises bagasse and a dry inorganic salt; and the slurry comprises a polycationic material in the range of about 1%-4% by weight.

A lid manufactured according to the foregoing methods is also provided.

In an embodiment the lid further includes a lock ring having a non-positive draft.

A vacuum tool is also provided for manufacturing a fiber-based beverage lid having a crown and a lock ring including a negative draft. The tool includes: a mold block supporting a lock ring mold portion corresponding to the lid lock ring; a retractable piston assembly comprising a crown mold portion corresponding to the lid crown and a piston shaft; and a pneumatic actuator configured to extend the piston shaft to thereby remove the lid lock ring from the lock ring mold portion.

In an embodiment the vacuum tool further includes a wire mesh removably surrounding the crown mold portion and the lock ring mold portion.

A shipping container kit is also provided for a flat screen TV. The kit includes: a top cover; a screen protector; four corrugated pulp corner pieces configured to fit over respective corresponding corners of the flat screen TV; a bottom tray configured to nest with the top cover; and a pallet strap configured to secure the TV, screen protector, corrugated pulp corner pieces within the nested top cover and bottom tray.

In an embodiment, the corrugated pulp corner pieces are manufactured using a slurry comprising at least one of: softwood (SW); bagasse; bamboo; old corrugated containers (OCC); and newsprint (NP).

A packing system is also provided for shipping original design manufacturer (ODM) boxes. The system includes: a plurality of corner sets, each comprising at least two fiber cushions; a plurality of end cap sets, each comprising two opposing corrugated sleeves; and a graphical guide comprising and end cap selector and a corner selector

## 18

In an embodiment, the graphical guide is configured to allow a user to: compare an ODM box to the end cap selector to thereby select one of the plurality of end cap sets; and compare the ODM box to the corner selector to thereby select one of the plurality of end corner sets.

In an embodiment, each sleeve comprises a plurality of height score lines, a plurality of width score lines, and a support feature to stabilize the sleeve during folding.

In an embodiment, each of the plurality of corner sets are 10 vacuum formed from a fiber-based slurry.

In an embodiment, the plurality of corner sets comprises at least a first corner set having four fiber cushions of a first size, and a second corner set having four fiber cushions of a second size; and the plurality of end cap sets comprises at 15 least a first end cap set having two sleeves of a first size, and a second end cap set having tow sleeves of a second size.

In an embodiment, the plurality of corner sets further comprises a third corner set having four fiber cushions of a third size, and a fourth corner set having four fiber cushions of a fourth size; and the plurality of end cap sets further comprises a third end cap set having two sleeves of a third size.

In an embodiment, the end cap selector comprises a first 25 zone corresponding to the first end cap set, and a second zone corresponding to the second end cap set; and the corner selector comprises a first guide line corresponding to the first corner set, and a second guide line corresponding to the second corner set.

In an embodiment, the plurality of height score lines are 30 configured to allow a user to select a particular one of the height score lines based on the height of the ODM box, and to fold the sleeve along the selected height score line; and the plurality of width score lines are configured to allow a user to select a particular one of the width score lines based 35 on the width of the ODM box, and to fold the sleeve along the selected width score line.

In an embodiment, the support feature comprises a plurality of tabs, each corresponding to a respective width score line.

In an embodiment, the system further includes a generally 40 u-shaped corrugated screen protector comprising an array of vacuum molded fiber feet.

In an embodiment, each of the first size corner cushions 45 comprises a first width corresponding to a first one of the width score lines; and each of the second size corner cushions comprises a second width corresponding to a second one of the width score lines.

In an embodiment, the system is configured to be 50 assembled such that: the screen protector is disposed over the top of the ODM box, with the array of feet adjacent a front surface of the ODM box; a top corner of each sleeve, when folded along the selected width score line and the selected height score line, mates with a corresponding top 55 corner of the ODM box, with one of the selected corner cushions disposed therebetween; and a bottom corner of each sleeve, when folded along the selected width score line and the selected height score line, mates with a corresponding bottom corner of the ODM box, with one of the selected corner cushions disposed therebetween.

In an embodiment, system of claim 1, is further configured to be secured in the assembled position for shipping using at least one of stretch paper and pallet straps.

A method of packing an original design manufacturer 60 (ODM) box is also provided. The method includes: providing a plurality of corner sets, each comprising at least two fiber cushions; providing a plurality of end cap sets, each

## 19

comprising two opposing corrugated sleeves; and providing a graphical guide comprising an end cap selector and a corner selector.

In an embodiment, the graphical guide is configured to allow a user to: compare an ODM box to the end cap selector to thereby select one of the plurality of end cap sets; and compare the ODM box to the corner selector to thereby select one of the plurality of end corner sets; and further wherein each sleeve comprises a plurality of height score lines, a plurality of width score lines, and a support feature to stabilize the sleeve during folding. 10

In an embodiment, each of the plurality of corner sets are vacuum formed from a fiber-based slurry.

In an embodiment, the plurality of corner sets comprises at least a first corner set having four fiber cushions of a first size, and a second corner set having four fiber cushions of a second size; the plurality of end cap sets comprises at least a first end cap set having two sleeves of a first size, and a second end cap set having two sleeves of a second size; the end cap selector comprises a first zone corresponding to the first end cap set, and a second zone corresponding to the second end cap set; and the corner selector comprises a first guide line corresponding to the first corner set, and a second guide line corresponding to the second corner set. 15 20

In an embodiment, the method further comprises: selecting a particular one of the height score lines based on the height of the ODM box, and folding the sleeve along the selected height score line; and selecting a particular one of the width score lines based on the width of the ODM box, and folding the sleeve along the selected width score line. 25

In an embodiment, the method further comprises: placing a screen protector over the top of the ODM box with an array of fiber feet adjacent a front surface of the ODM box; mating a top corner of each sleeve with a corresponding top corner of the ODM box, with one of the selected corner cushions disposed therebetween; and mating a bottom corner of each sleeve with a corresponding bottom corner of the ODM box, with one of the selected corner cushions disposed therebetween. 30 35

In an embodiment, the method further comprises securing the assembled ODM box, screen protector, end caps, and corner cushion for shipping using at least one of stretch paper and pallet straps.

As used herein, the word "exemplary" means "serving as an example, instance, or illustration." Any implementation described herein as "exemplary" is not necessarily to be construed as preferred or advantageous over other implementations, nor is it intended to be construed as a model that must be literally duplicated.

While the foregoing detailed description will provide those skilled in the art with a convenient road map for implementing various embodiments of the invention, it should be appreciated that the particular embodiments described above are only examples, and are not intended to limit the scope, applicability, or configuration of the invention in any way. To the contrary, various changes may be made in the function and arrangement of elements described without departing from the scope of the invention. 50 55

The invention claimed is:

1. A packing system for shipping original design manufacturer (ODM) boxes, the system comprising:  
a plurality of corner sets, each vacuum formed from a fiber-based slurry and each comprising at least two fiber cushions;  
a plurality of end cap sets, each comprising two opposing corrugated sleeves; and

## 20

a graphical guide comprising an end cap selector and a corner selector;

wherein:

the graphical guide is configured to allow a user to: i) compare an ODM box to the end cap selector to thereby select one of the plurality of end cap sets; and ii) compare the ODM box to the corner selector to thereby select one of the plurality of end corner sets; each sleeve comprises a plurality of height score lines, a plurality of width score lines, and a support feature to stabilize the sleeve during folding;

the plurality of corner sets comprises at least a first corner set having four fiber cushions of a first size, and a second corner set having four fiber cushions of a second size, wherein the first size is different from the second size; and

the plurality of end cap sets comprises at least a first end cap set having two sleeves of a first size, and a second end cap set having two sleeves of a second size.

## 2. The system of claim 1, wherein:

the plurality of corner sets further comprises a third corner set having four fiber cushions of a third size, and a fourth corner set having four fiber cushions of a fourth size; and

the plurality of end cap sets further comprises a third end cap set having two sleeves of a third size.

## 3. The system of claim 1, wherein:

the end cap selector comprises a first zone corresponding to the first end cap set, and a second zone corresponding to the second end cap set; and

the corner selector comprises a first guide line corresponding to the first corner set, and a second guide line corresponding to the second corner set.

## 4. The system of claim 3, wherein:

the plurality of height score lines are configured to allow a user to select a particular one of the height score lines based on the height of the ODM box, and to fold the sleeve along the selected height score line; and

the plurality of width score lines are configured to allow a user to select a particular one of the width score lines based on the width of the ODM box, and to fold the sleeve along the selected width score line.

5. The system of claim 4, wherein the support feature comprises a plurality of tabs, each corresponding to a respective width score line.

6. The system of claim 4, further comprising a generally u-shaped corrugated screen protector.

7. The system of claim 6, wherein the screen protector comprises an array of vacuum molded fiber feet.

## 8. The system of claim 4, wherein:

each of the first size corner cushions comprises a first width corresponding to a first one of the width score lines along which the end cap is to be folded; and

each of the second size corner cushions comprises a second width corresponding to a second one of the width score lines along which the end cap is to be folded.

9. The system of claim 8, configured to be assembled such that:

the screen protector is disposed over the top of the ODM box, with the array of feet adjacent a front surface of the ODM box;

a top corner of each sleeve, when folded along the selected width score line and the selected height score line, mates with a corresponding top corner of the ODM box, with one of the selected corner cushions disposed therebetween; and

a bottom corner of each sleeve, when folded along the selected width score line and the selected height score line, mates with a corresponding bottom corner of the ODM box, with one of the selected corner cushions disposed therebetween.

\* \* \* \* \*